

## UNITED STATES PATENT OFFICE

1,987,530

## EXPANSION JOINT FILLING MATERIAL

John S. Hippel, Temple, Pa.

No Drawing. Application March 17, 1931,  
Serial No. 523,376

9 Claims. (Cl. 106—31)

This invention relates generally to materials, applicable than known similar substances, and for filling expansion joints and particularly to an improvement in such materials which results in its having the features of novelty and advantage, set out in detail below.

It is an object of this invention to provide a material of the type described which will not only fulfill the ordinary requirements of a material of this character, but which will have the additional advantages of remaining soft and pliable at very low temperatures, and remaining plastic and full-bodied at temperatures ranging up to 200 degrees Fahrenheit.

It is also an object of this invention to provide a material of the character described which will have very little variation at high and low temperatures as respects a penetration test, in contrast to the extensively used asphalt and tar materials which show under the penetration test, impenetrability at low temperatures, and complete loss of plasticity and elasticity and body at higher temperatures.

It is also an object of this invention to provide a material of the character described which while efficiently and very satisfactorily resisting the action of the elements when used outdoors, will have the additional advantage of resisting chipping at low temperature, since at low temperatures it retains its softness and pliability as well as elasticity.

It is a further object of this invention to provide a material of the character described which is adaptable to take the place of such materials and structures which have heretofore been used, particularly in filling the expansion joints in roads particularly of the concrete type, but which may be used in any place or structure requiring a resilient, elastic, and plastic material, which will retain its form and condition in spite of variations within wide ranges of temperature.

It is also an object of this invention to provide a material of the character described which is ideally adapted to function as a filler for the expansion joints of concrete road constructions and which at high temperatures may be poured into the said expansion joints and which upon cooling, forms the required weatherproof and moisture-proof joint responsive to the expanding and contracting movement of the concrete and the like constituting the joint.

It is a further object of this invention to provide a material of the type described which is composed of a new and novel combination of elements, which renders the material more satisfactory, more durable, and above all more easily

These and other objects of the invention, its nature, and its composition and arrangement and combination of parts will be readily understood by any one acquainted with the art to which this invention relates upon consulting the following descriptions and explanations.

Although, at the present time, various substances are used for forming expansion joints of the type described, it is well known that they very imperfectly fulfill the requirements, especially when used to form expansion joints in concrete roadways and other construction work. Presently used substances with few if any exceptions exhibit a positive tendency to project above the road surface, under squeezing action of the concrete or other material so that the portion thus protruding is struck continuously by passing vehicles. Further, the protruding portion of the substance is subject to be chipped or broken in cold weather, and spread and tracked over the road surface in warm weather, due to brittleness at low temperatures and loss of body at high temperatures. Further, due to the changed condition of such substances at the extremes of temperatures they fail to adhere properly to the sides of the concrete or other substance, and so fail to form a weather proof joint.

Besides being strongly adhesive, the material of my invention will not chip in a circumstance similar to that mentioned above at a temperature in the neighborhood of below zero, and it will not run or lose its body, nor its plasticity, nor its elasticity, at temperatures ranging up to 200 degrees Fahrenheit. The result is that the annoyances and expenses alluded to are eliminated when the material of my invention is used as a joint filler of the type described. It should be understood that various other types of expansion joints, not included in the concept of concrete road expansion joints, may be successfully packed with my improved material, at a less expense for installation and for upkeep.

A soft, elastic, plastic, pliable, material having the resistive quality noted above is, according to my invention produced by oxidizing and vulcanizing vegetable and fish oils, such as olive oil, corn oil, palm oil, rapeseed oil, fish oil, linseed oil, cotton seed oil, menhaden oil or any unsaturated fats or fatty oils capable of being oxidized or vulcanized. The use of any or a combination of any

5

10

15

20

25

30

35

40

45

50

55

of the above oils and fats, may be selectively made with a view to employing the least expensive thereof, whereby the cost of the final product may be reduced, and its use thereby rendered more economical than in the case with the well known asphaltum, tar, and hydrocarbon materials now in extensive use for the same or for similar purposes. It will be observed that some of the above oils, are known in the art as drying, or semidrying oils, such as particularly cottonseed oil, linseed oil, and rapeseed oil.

A very satisfactory formula for use in making a batch of my improved expansion joint filling material for use in filling the expansion joints of concrete road constructions is as follows, it being understood that any of the vegetable oils, fats or oxidizable or vulcanizable fats and oils mentioned above may be substituted for the oils mentioned in the formula, as well as others.

20 The formula:—

8 parts cottonseed oil, 8 parts linseed oil, 8 parts sulphur, 4 parts rosin, 4 parts pulverized mineral such as silica, clay, talc, etc., 1 part "Hydrolene", being the trade name for a petroleum pitch produced by aerating residual oils, 1 part of a

30 One method of making the product of the invention from the foregoing ingredients consists of heating the stated proportions of cottonseed oil, linseed oil, rosin, and "Hydrolene" in an iron kettle under an open flame to about 200 degrees centigrade, or until the rosin and "Hydrolene" are liquefied. Upon the appearance of this phenomenon, the pulverized silica and sulphur is added. The heating is continued until the vulcanization and other re-actions have begun, at which point the heat is withdrawn, and the product permitted to cool, and it is then poured into suitable molds, or into the expansion joints to be filled.

40 It will be understood as stated herein, that the method contemplates the performance of the same steps if oils other than cottonseed oil and linseed oil are employed in the stead of the cottonseed oil and linseed oil mentioned in the statement of the method.

50 A statement of the method or process herein appearing also appears in my Letters Patent 1,888,270 issued November 22, 1932.

55 It is to be definitely understood that I do not desire to limit the application of this invention to the particular modification set out herein to illustrate the principles thereof, and any change or changes may be made in materials and ingredients and in their proportions, and quantities and in the sequence and duration of operations and steps involved in their assembly or agglom-

60 eration of the material, and to any other modification which may be suggested to one skilled in the art, and which may be made without departing from the spirit and scope of the invention.

erations, within the spirit and scope of the invention.

What is claimed is:—

1. An expansion joint filling material which retains substantially its plasticity, body, and cohesiveness at temperatures ranging from 0° to 200° Fahrenheit, comprising the reaction product of substantially equal proportions of vegetable oil, of drying oil, and of a vulcanizing agent; and substantially smaller proportions of rosin and of silica, and about 3% of blown asphalt.

2. An expansion joint filling material which retains substantially its plasticity, body, and cohesiveness at temperatures ranging between 0° and 200° Fahrenheit, comprising the reaction product of eight parts of vegetable oil, eight parts of drying oil, eight parts of a vulcanizing agent, four parts of rosin, four parts of pulverized silica, and one part of blown asphalt.

3. An expansion joint filling material which retains its adhesiveness, plasticity, body, and cohesiveness through a wide range of temperatures, comprising the reaction product of eight parts of cotton seed oil, eight parts of linseed oil, eight parts of sulphur, four parts of rosin, four parts of pulverized silica, and not over 3% of Hydro-

lene.

4. An expansion joint filling material comprising the reaction product of substantially equal portions of a vulcanizable fat, of a vegetable drying oil, and of sulphur, a smaller quantity of rosin, and a quantity of pulverized mineral equal to the quantity of rosin.

5. An expansion joint filling material comprising the reaction product of substantially equal proportions of a vulcanizable organic oil, of vegetable drying oil, and of sulphur, together with smaller proportions of rosin and pulverized silica.

6. An expansion joint filling material comprising the reaction product of approximately, 16 parts of vulcanizable vegetable oil, 8 parts of a vulcanizing agent, 4 parts of rosin, 4 parts of silica, and 1 part of blown asphalt.

7. An expansion joint filling material composed of the reaction product of approximately, 16 parts of a mixture of vulcanizable vegetable oils, 8 parts of a vulcanizing agent, 4 parts of rosin, 4 parts of silica, and 1 part of blown asphalt.

8. An expansion joint filling material composed of the reaction product of 8 parts of cottonseed oil, 8 parts of linseed oil, 8 parts of sulphur, 4 parts of rosin, 4 parts of silica, and 1 part of blown asphalt.

9. An expansion joint filling material composed of the reaction product of 16 parts of a mixture of cottonseed oil and linseed oil, 8 parts of sulphur, 4 parts of rosin, 4 parts of silica, and 1 part of blown asphalt.

JOHN S. HIPPLE.